

July 23, 1957

W. M. DUNCAN

2,799,906

APPARATUS AND METHOD OF FILLING INGOT MOLDS

Filed Jan. 26, 1953



FIG. 1.



FIG. 2.

INVENTOR,  
WILLIAM M. DUNCAN,

BY  
*Browning and Letherland*,  
ATTORNEYS.

**1**

2,799,906

**APPARATUS AND METHOD OF FILLING INGOT MOLDS**

William M. Duncan, Alton, Ill.

Application January 26, 1953, Serial No. 333,317

2 Claims. (Cl. 22—155)

This invention relates to methods of and apparatus for pouring ingots.

One of the principal problems confronting the industry has been that of preventing piping or spongy spots from occurring in the center of ingots. It will be understood that when metal poured into an ingot mold freezes, there is a reduction in volume or shrinkage of crystallization, which tends to produce voids in the center portions of the casting. Such voids result in structural weakness when the ingot is later worked, as by forging or the like. Accordingly, it is an object of this invention to avoid formation of such piping in pouring ingots. Another object of the invention is to provide for continuous pouring of ingots, using conventional open-top ingot molds.

In accordance with this invention, briefly stated, molds are arranged in a row and are connected together at their sprues by inclined runners. Once a mold is filled, liquid metal is caused to flow over its sprue to feed shrinkage therein, while the excess metal over that required to feed shrinkage is directed by the runner into a next mold. More particularly, conventional open-top ingot molds are carried on cars moved along an inclined track leading up to the pouring station. A refractory covering is placed on top of the molds to form a continuous runner extending the length of the train, with sprues opening from the runner into the mold cavity. Metal is then poured in the runner adjacent to the upper end of its incline to fill molds as they are moved to the pouring point, and feed shrinkage in a filled mold as it moves beneath the pouring point.

Pouring is preferably continuous, but the first mold is not moved from beneath the ladle immediately upon being filled. Instead, metal is poured or caused to flow over the associated sprue for a substantial length of time thereafter, the overflow being directed by the runner to fill a following mold. The mold movement may be continuous, but any given mold should be filled before its arrival at the pouring point so that there is an opportunity to feed shrinkage from the runner before the mold moves beyond the pouring point. In this way, an adequate supply of liquid metal for feeding shrinkage in the mold proper is not only assured, but heat is supplied to the metal in a sprue opening so as to prevent premature freezing of metal at the sprue.

Other features of the invention will be in part apparent from and in part pointed out in the following detail description taken in connection with the accompanying drawings, in which:

Fig. 1 is a top plan view illustrating the invention as employed in pouring ingots; and,

Fig. 2 is a side elevation of the apparatus shown in Fig. 1, parts being shown in section.

Referring now to the drawings, molds 1 are arranged in a row for relative movement with respect to a pouring station. In the illustrated embodiment, the molds are carried by trucks 3, which are coupled together at 7 in uniformly spaced relationship, and the trucks are moved along a track 5 in the direction indicated by a suitable de-

**2**

vice (not shown). The molds 1 are conventional ingot molds, with cavities 9 and relatively large open tops 11 through which the finished ingots are removed. As such, the system is similar to that presently in use. In contrast to prior practice, however, the track 5 is on a slight incline, at least in part, in the direction of mold movement, and the molds are connected together at their tops by runners. The runners may be formed by covers or lids 13, which are generally flat rectangular members of refractory material. A groove 15 in the upper surface of each member functions to channel flow of liquid metal between walls 17, and at the ends of the groove are recesses 19, which form relatively small sprue openings for filling the molds.

In operation, the covers 13 are arranged in end-abutting relationship on top of the molds, each member 13 reaching from the center of one mold to the center of an adjoining mold. The molds are thus closed except for relatively small sprue openings 19 which are connected together by a continuous runner extending the length of the train. Metal is poured into the runner from a ladle 21 or other source of liquid metal located at a point adjacent the upper end of the inclined part of the track.

At the beginning of a pouring operation, the initial mold is moved generally beneath the ladle 21 and filled. When filled, the mold is not immediately moved from beneath the ladle, but liquid is allowed to flow onto or over the associated sprue while the metal in this initial mold cools and sets. Consequently, a continuous supply of hot liquid metal is present at the sprue to feed whatever shrinkage occurs, the excess over that required to feed shrinkage being directed by the runner 15 into a following mold. After the possibility of shrinkage at the first mold has passed, the molds may be moved continuously as a unit until the pouring operation is completed.

During movement of the molds, metal continues to flow from the ladle, but it will be apparent that the molds are filled before they reach the ladle. In other words, a given mold arriving at the pouring station 23 has been filled previously from the runner 15, and shrinkage is in progress; however, such shrinkage is adequately fed from the runner as the mold moves to and beneath the ladle.

As the last mold in the train approaches the ladle, the pouring may be stopped, in which event some shrinkage will occur in the final ingot, but that ingot may be remelted. After the pouring operation has been completed, the covers 13 are removed from the molds to permit withdrawal of the ingots.

The rate of flow at 23 and the rate of mold movement are controlled relative to one another so as to maintain a stabilized condition during the pouring operation; and both metal flow and mold movement are adjusted relative to the time required for the metal in a filled mold to freeze. For example, the time required for the metal in a mold to set after filling, the time required to fill mold C-1 and feed shrinkage at B-1 (as determined by the rate of flow at 23), and the time required for mold C-1 to move to the ladle after filling (as determined by the speed of the trucks 3), should all be approximately equal.

From the foregoing description, it is apparent that those skilled in the art will understand the structure, methods, function, and mode of operation of the invention herein disclosed, and appreciate the advantages thereof. It may be noted, that whereas the invention is described in particular as utilized in the pouring of ingots, the invention may also be used in pouring other types of castings, and reference is made by my copending application entitled Manufacture of Castings, Serial No. 333,316, filed January 26, 1953.

Although one embodiment has been disclosed in de-

tail, it is to be understood that the invention is not limited thereto, but the drawings and description thereof are to be understood as being merely illustrative.

It is realized that other modifications and variations will present themselves to those skilled in the art without departing from the spirit of this invention or the scope thereof as set forth in the appended claims.

Having thus described the invention, what is claimed and desired to be secured by Letters Patent is:

1. Apparatus for filling conventional open-top ingot molds comprising a track inclined to a pouring station, a plurality of cars on said track, each of said cars carrying an ingot mold, and re-usable cover sections laid in end-abutting relationship on top of and bridging adjacent molds, said cover sections being shaped to form an open trough extending lengthwise of the train with sprues opening therefrom into said molds at the abutting ends of said cover sections.

2. A re-usable cover section for use in pouring ingots with conventional open-top ingot molds which are carried on a train of cars, said cover section being formed of refractory material and being of a length sufficient to extend between the centers of adjacent cars and of a width sufficient to cover the top of an ingot mold, said cover section having a groove extending lengthwise from end to end, and a sprue-forming recess extending across one end thereof from said groove.

References Cited in the file of this patent

UNITED STATES PATENTS

|           |               |       |               |
|-----------|---------------|-------|---------------|
| 521,449   | Adams         | ----- | June 19, 1894 |
| 735,303   | Sauver        | ----- | Aug. 4, 1903  |
| 1,454,741 | Howard et al. | ----- | May 8, 1923   |
| 1,572,866 | McKune        | ----- | Feb. 9, 1926  |
| 2,326,164 | Payne         | ----- | Aug. 10, 1943 |